

## UNITED STATES PATENT OFFICE

2,077,073

## RECOVERY OF METALS FROM THEIR ORES

Manley L. Ross, Niagara Falls, N. Y., assignor to  
E. I. du Pont de Nemours & Company, Wilming-  
ton, Del., a corporation of Delaware

No Drawing. Application August 1, 1934, Serial  
No. 737,929

6 Claims. (Cl. 23—18)

This application relates to a process of recovering metals from their ores and more particularly to a process in which sulfur chloride is employed in converting the metallic constituent of the ore into a form in which the metal can be recovered. The process is of greatest utility in recovering tungsten from its ores as tungsten trioxide.

Previously when any of the sulfur chlorides, such as the monochloride or dichloride or a mixture of sulfur chlorides, were employed in the recovery of metals from their ores, it was necessary to carry out the treatment at a relatively high temperature and in the vapor phase. It has now been found that the metal present in the ore can be readily digested by sulfur chloride and converted to a form in which it is readily soluble at a temperature below the boiling point simply by refluxing the ore and the extracting liquid.

The chlorides of sulfur have been used to some extent in metallurgy for converting the metals present in the ores into chlorides and oxy chlorides in which form the metallic constituent can be readily recovered. However, all of these prior processes have found it necessary to employ relatively high temperatures and sulfur chloride or a mixture of sulfur chloride and chlorine in the gaseous phase. Thus, the prior art indicates that tungsten can be recovered by passing sulfur chlorides and chlorine over a wolframite at a temperature of about 200° C. At this temperature, by the use of the extracting medium in the gaseous phase, it has been found that substantially all the tungsten is converted to a soluble form while at the same time a small amount is volatilized. In general, prior methods have found it necessary to work with sulfur chloride and chlorine at a temperature just under the temperature at which the tungsten is volatilized, which is in the neighborhood of 230° C. This relatively high temperature has been previously considered necessary in order to render the greater portion of the tungsten soluble when that metal is being recovered from its ores.

It is especially advantageous to convert the metal in the ore into a soluble form permitting ready recovery by the use of an extracting medium in the liquid phase. By the use of a relatively low temperature, one which is below the boiling point of the sulfur chloride or mixture of sulfur chlorides which are used, losses due to volatilization of the tungsten or other metal being recovered are entirely avoided. In addition, by the use of liquid phase methods it is possible to carry out the reaction without the necessity of providing pressure-resistant apparatus or without having to maintain a high working temperature during the recovery process.

It has also been necessary in the prior art

where sulfur chlorides have been used in ore treatment, first to ignite the ore in a furnace for two to three hours in order to render it sufficiently soluble to permit recovery of the metal in economically important yields. By carrying out the step of extracting the metal from the ore in the liquid phase I have found that this preliminary treatment is unnecessary and yields of 91-92%, or higher, based upon the tungsten content of the ore, are readily obtained without preliminary ignition.

Throughout this description and in the claims I shall refer to the material used for digesting the ore as "sulfur chloride" although in practice it is well recognized that one or more chlorides of sulfur may be present in admixture. It has been found most convenient to prepare the sulfur chloride by passing chlorine over molten sulfur at a temperature of 140-150° C. The sulfur chloride passes off as vapor and is condensed to recover the liquid. The product is usually a mixture of  $S_2Cl_2$  and  $SCl_2$  but the ratio of one component to the other in the product is not known. The boiling point of the condensed liquid has been found to range from 50-138° C.

Throughout this specification the novel and improved process for the recovery of metals from their ores will be described using tungsten and tungsten ores as the examples. Although other metals may be recovered from their ores by the use of my process, I have found that the method is particularly suitable for tungsten recovery because of the relatively high degree of insolubility of its oxide in the customary digestion media.

The ore to be extracted, which may be wolframite when tungsten is being recovered, is first ground up into small pieces. I have found that grinding to a fineness of 200 mesh is usually very satisfactory. The ore is next digested by refluxing with sulfur chloride and chlorine at a temperature below the boiling point, within the range 50-138° C. I have found that a temperature within the range 125-138° C. is preferable although lower temperatures, of 50° C. or higher may be employed with very satisfactory results.

Excellent results have been obtained by utilizing about 125 parts by weight of sulfur chloride to 50 parts by weight of the wolframite ore. The digestion may be carried out for periods of from 4 to 7 hours in an atmosphere of chlorine. The ore, sulfur chloride, and chlorine are preferably held at the refluxing temperature for the desired period of time (4-7 hours) and chlorine gas may be fed slowly over the mixture. It is not essential that chlorine be present as sulfur chloride alone is effective; however the digestion probably proceeds more rapidly with chlorine present with the sulfur chloride.

The yield of tungstic acid obtained by this

method has been found to depend upon three factors: (1) fineness of division of the ore, (2) time of digestion, and (3) quantity of sulfur chloride used. The relative amounts of reagents, fineness 5 of the ore, and digestion period given above will be found to yield very satisfactory results.

After digestion the excess sulfur chloride in the mixture is distilled off and the hydrolyzable chlorides and monochlorides are hydrolyzed by boiling 10 with water. This treatment breaks down the chlorides to an insoluble metal compound as for example tungstic acid when tungsten is being recovered.

The gangue may then be filtered to free it of 15 the acid soluble salts which are present as impurities and whose recovery is not desired, such as those of manganese and iron. The gangue should then be washed free of the remaining acid soluble salts, particularly the chlorides of iron and 20 manganese, with dilute hydrochloric acid. The metal remains as an insoluble compound in the gangue.

The next step in my process is to treat the gangue with ammonium hydroxide, aqua-ammonia. 25 This converts the insoluble metal compound, which is tungstic acid when tungsten is being recovered, into an ammonium salt of the metal. The extract after treatment of the gangue with the ammonium hydroxide is then evaporated to 30 dryness and/or ignited. This treatment results in the recovery of the metal in the form of the metal oxide. When tungsten ores are being treated yields of 90-92%, based on the tungsten in the ore, are readily obtained.

That portion of the metal which remains in the gangue may be recovered therefrom by nitric acid 35 digestion and recovered by way of the ammonium salt of the metal. Evaporation to dryness and ignition will yield the desired metal oxide and by utilizing nitric acid to regain the small amounts of 40 metal remaining, yields of over 99%, based on the metal content of the ore, are not unusual when tungsten ore is being treated.

It will be readily appreciated that by digesting 45 the ore with sulfur chloride and chlorine in the liquid phase at relatively low temperatures a distinct improvement has been made in metal recovery methods. The use of high temperatures, and of apparatus which must be specially designed to 50 resist high temperatures and working in the vapor phase, is no longer necessary. The yields obtained by digestion in the liquid phase are as high, if not higher than those which may be obtained by vapor phase recovery methods.

As an example of my novel process applied to 55 the recovery of tungsten from its ore, numerical results illustrating two typical runs are tabulated below. As previously stated, tungsten is taken merely as illustrative and my method might be 60 used equally as well in the recovery of other metals.

A typical tungsten ore will analyze as follows:

|                        | Percent       |
|------------------------|---------------|
| WO <sub>3</sub> -----  | from 73 to 75 |
| FeO -----              | from 9 to 11  |
| MnO -----              | from 12 to 14 |
| CaO -----              | from 0 to 1   |
| SiO <sub>2</sub> ----- | from 0 to 1   |

This is a typical wolframite ore and from the analysis it is apparent what impurities are ordinarily present.

#### Example I

The ore, a sample of wolframite, was ground

and screened to a fineness of 200 mesh. A 50 gram sample was placed in a 1 liter, 3-necked flask and a quantity of sulfur chloride which varied from 75 cc. to 150 cc. was added. The sulfur chloride was prepared by passing chlorine over molten sulfur at 140°-150° C. and then condensing the effluent vapors.

The liquid and ore were refluxed for from 4-7 hours, the temperature being maintained below 138° C. Chlorine gas was slowly fed over the surface of the mixture during the digestion.

After digestion water was added to the mixture and the contents were boiled in order to hydrolyze the remaining sulfur chloride and break down the chlorides and oxychlorides of tungsten present in the mixture to tungstic acid. The gangue was next washed free of the acid soluble salts which would otherwise be present as iron and manganese impurities in the product by treatment with dilute hydrochloric acid.

Sufficient ammonium hydroxide is then added to render the mass ammoniacal and the extract separated from the gangue by filtration. This extract contained the tungsten as an ammonium salt and was evaporated to dryness and ignited. The yield of tungsten based on the quantity of the metal in the ore was 91-92%, the digestion period having been 7 hours.

The gangue was then treated with nitric acid in order to recover the remaining tungsten. To the extract ammonium hydroxide was added and the solution evaporated to dryness. The total recovery of tungstic acid was 97-99.6% based on the metallic content of the ore.

The following numerical values indicate the relative proportions of reagents and amounts in two typical runs:

|                                                                                             | Run 1 | Run 2 | 40 |
|---------------------------------------------------------------------------------------------|-------|-------|----|
| Wt. of ore in grams-----                                                                    | 50.00 | 50.00 |    |
| Vol. of sulfur chloride in cc.-----                                                         | 150   | 75    |    |
| Time of digestion in hours-----                                                             | 7     | 7     |    |
| Wt. of WO <sub>3</sub> in ore, grams-----                                                   | 26.40 | 26.40 |    |
| Wt. of WO <sub>3</sub> recovered by sulfur chloride treatment, grams-----                   | 24.30 | 24.10 | 45 |
| Wt. of WO <sub>3</sub> remaining and recovered by HNO <sub>3</sub> digestion, in grams----- | 2.03  | 1.55  |    |
| Total WO <sub>3</sub> acent. for, in grams-----                                             | 26.33 | 25.65 |    |
| % yield of WO <sub>3</sub> without HNO <sub>3</sub> digestion-----                          | 92.0  | 91.5  |    |
| % WO <sub>3</sub> remaining and acent. for by HNO <sub>3</sub> digestion-----               | 7.6   | 5.9   |    |
| Total yield of WO <sub>3</sub> in %-----                                                    | 99.6  | 97.2  | 50 |

It is obvious that various changes might be made in the described method of recovering metals from their ores without departing from the principles herein set forth. The various manipulative details given in describing my preferred embodiment are to be considered merely as illustrative and not restrictive, and various modifications might be made therein without departing from the spirit of my invention.

I claim:

1. A process of recovering tungsten from its ores in the form of tungsten oxide which comprises the steps of refluxing the ore with sulfur chloride in the liquid phase at a temperature within the range 50 to 138° C., treating the resulting product with water to hydrolyze the tungsten compounds present in the gangue, adding aqua ammonia to render the tungsten compounds soluble, filtering said tungsten compounds from the gangue, and then evaporating the filtrate to dryness to recover the tungsten.

2. A process of recovering tungsten from its ores in the form of tungsten oxide which comprises the steps of refluxing the ore with sulfur chlo-

ide in the liquid phase in the presence of chlorine at a temperature of 50 to 138° C., treating the resulting product with water to hydrolyze the tungsten compounds present in the gangue, adding aqua ammonia to render the tungsten compounds soluble, filtering the tungsten from the gangue, evaporating the filtrate to dryness to recover the tungsten, and treating the gangue with nitric acid to recover additional tungsten.

10 3. A process for recovering tungsten from its ores in the form of tungsten oxide which comprises the steps of refluxing the ore with sulfur chloride in the liquid phase in the presence of chlorine at a temperature within the range 50 to 138° C., treating the resulting product with water to hydrolyze the tungsten compounds present in the gangue, washing the gangue with dilute hydrochloric acid to free it of acid soluble salts, filtering, adding aqua ammonia to render 20 the tungsten compounds present in the gangue soluble, filtering the tungsten from the gangue, evaporating the filtrate to dryness to recover the tungsten, and subsequently recovering additional tungsten by treating the gangue with an acid.

25 4. A process of recovering tungsten from its ores in the form of tungsten oxide which comprises the steps of grinding the ore into fine particles, refluxing said ore with sulfur chloride in the liquid phase in the presence of chlorine at 30 a temperature of 50-138° C., treating the resulting product with water to hydrolyze the tungsten compounds present in the gangue, washing the mixture with a dilute acid to free it from acid soluble salts, filtering, treating the gangue 35 and tungsten mixture with aqua ammonia in order to render the tungsten soluble, filtering, evaporating the filtrate to dryness and igniting in order to recover the tungsten as tungsten oxide, treating the gangue with nitric acid to recover any remaining tungsten, filtering.

adding aqua ammonia to the filtrate, and then evaporating to dryness to separate the additional tungsten as tungsten oxide.

5. A process of recovering tungsten from its ore in the form of an oxide of tungsten which comprises the steps of refluxing the ore with sulfur chloride in the liquid phase in the presence of chlorine at a temperature of 125-138° C., treating the resulting product with water to hydrolyze the tungsten compounds present in the gangue, adding aqua ammonia to render the tungsten compounds soluble, filtering the tungsten from the gangue, evaporating the filtrate to dryness to recover the tungsten as the tungsten oxide, and then treating the gangue with an acid 10 to recover additional metal.

6. A process of recovering tungsten from its ores in the form of the oxide which comprises the steps of comminuting the ore, refluxing said ore with sulfur chloride in the liquid phase in the presence of chlorine for 4 to 7 hours at a temperature of 125-138° C., treating the resulting product with water to hydrolyze the tungsten compounds present in the gangue, washing the mixture of gangue and tungsten compound with dilute hydrochloric acid in order to remove the acid soluble salts, filtering, treating said mixture of tungsten compounds and gangue with aqua ammonia in order to render the tungsten soluble, filtering the tungsten compounds from the gangue, evaporating said filtrate to dryness and igniting to recover the tungsten in the form of the oxide, treating the gangue with nitric acid to recover additional tungsten, treating said mixture of gangue and tungsten compounds with aqua ammonia in order to render the tungsten soluble, filtering, and evaporating to dryness and igniting in order to recover the additional tungsten as the oxide.

MANLEY L. ROSS.

40